

## UNITED STATES PATENT OFFICE

2,224,151

## MAGNESIUM ALLOYS

Gaston Gauthier, Chambery, France, assignor to  
 "Compagnie de Produits Chimiques et Electro-  
 metallurgiques Alais, Froges et Camargue,"  
 Paris, France, a corporation of France

No Drawing. Application February 9, 1938, Se-  
 rial No. 189,645. In France February 16, 1937

4 Claims. (Cl. 75—168)

It is a well known disadvantage of magnesium base alloys that they are liable to progressive oxidation when in the molten state and that they are also subject to superficial oxidation when in the solid state, particularly at relatively high temperatures such as for instance higher than 5 300° C.

In order to reduce the liability of magnesium base alloys to oxidation it has been proposed to 10 incorporate small quantities of calcium in the alloys. It has also been suggested that the addition of small quantities of beryllium to such alloys reduces their liability to oxidation, and it is true that the effect of an addition of beryllium in 15 respect of this liability to oxidation is far more pronounced than that of corresponding amounts of calcium. On the other hand it has been observed that the incorporation of beryllium in magnesium or magnesium base alloys imparts to 20 the metal on solidification an extremely coarse-grain texture as compared with the corresponding metals in which beryllium is absent. Owing to this coarse-grain texture, the alloys containing beryllium have low mechanical strength 25 properties and particularly fatigue strength; moreover, when a thermal treatment of the metal or alloy is required, then the coarse-grain texture necessitates a much longer duration of such treatment than otherwise would be required.

30 It is an object of the present invention to provide magnesium base alloys containing beryllium in which the favourable known effects of beryllium as an inhibitor of oxidation are preserved, while at the same time avoiding the tendency to 35 coarse-grain crystallisation otherwise observable in magnesium alloys containing beryllium.

I have found that the presence of zirconium in magnesium base alloys containing beryllium has the effect of imparting thereto, on solidification, a fine-grain structure without in any way 40 impairing the resistance to oxidation due to the presence of the beryllium. At the same time, the joint presence of zirconium in the alloy avoids the undesirable reduction in mechanical properties imparted thereto by the presence of the beryllium, the mechanical strength properties being at least equal to those of the original metal or alloy containing neither beryllium nor zirconium.

50 By way of example, beryllium can be present in the metal or alloys in amounts lying between 0.005 and 0.5% while zirconium is present in amounts lying between 0.005 and 0.5%.

It has been found that a content of 0.025% of beryllium imparts to the alloy a sufficient re-

sistance to oxidation for all practical purposes, while a zirconium content of 0.05% is sufficient to counteract the disadvantages caused by the presence of that amount of beryllium in the alloy. 5

Based on the foregoing observations, the present invention provides a magnesium base alloy containing both beryllium and zirconium, preferably each in an amount lying between 0.005 and 0.5%. 10

The invention also provides a process of grain-refining magnesium base alloys containing beryllium, which consists in adding zirconium to said alloys.

The zirconium can be added either in making 15 up the alloys or when remelting ingots or scrap.

The zirconium may be introduced in any desired manner, for example in the form pre-alloys, or in the form of salts of zirconium which are adapted to be reduced to metal in contact with 20 the molten magnesium or magnesium base alloys.

The alloys of the present invention can even be melted without use of a flux. Due to the decreased liability to oxidation of the molten alloy, losses by burning are reduced to a minimum and 25 when no flux is used, salt inclusions in the metal, and therefore with their attendant risks of corrosion are impossible.

A further advantage arising out of the invention is that when subjecting the alloys to heat 30 treatment, the duration of the latter is the same as that for the same alloy, containing neither beryllium nor zirconium. In addition the parts subjected to the heat treatment do not become oxidised and retain their original lustre. 35

What I claim is:

1. A magnesium base alloy containing between about 0.005% and 0.5% beryllium and between about 0.005% and 0.5% zirconium characterized by a refined grain structure and by mechanical 40 properties at least equal to those of the same alloy without beryllium.

2. A magnesium base alloy containing about 0.025% beryllium and about 0.05% zirconium characterized by a refined grain structure and by 45 mechanical properties at least equal to those of the same alloy without beryllium.

3. A magnesium base alloy containing between about 0.005% and 0.5% beryllium and between about 0.005% and 0.5% zirconium, the balance 50 being substantially all magnesium.

4. A magnesium base alloy containing about 0.025% beryllium and about 0.05% zirconium, the balance being substantially all magnesium.

GASTON GAUTHIER. 55